

(No. Model.)

E. J. LUTWYCHE.  
ORNAMENTING GLASS.

No. 599,716.

Patented Mar. 1, 1898.



Witnesses

G. A. Bauberschmidt.  
D. Werner Reinohl.

Inventor

E. J. Lutwyche  
By D. C. Reinohl  
Atty.

# UNITED STATES PATENT OFFICE.

EDGAR J. LUTWYCHE, OF CHICAGO, ILLINOIS.

## ORNAMENTING GLASS.

SPECIFICATION forming part of Letters Patent No. 599,716, dated March 1, 1898.

Application filed April 15, 1897. Serial No. 632,201. (No model.)

*To all whom it may concern:*

Be it known that I, EDGAR J. LUTWYCHE, a citizen of the United States, residing at Chicago, in the county of Cook and State of Illinois, have invented certain new and useful Improvements in Ornamenting Glass; and I do hereby declare the following to be a full, clear, and exact description of the invention, such as will enable others skilled in the art to 10 which it appertains to make and use the same.

My present invention relates to the manufacture of glass, and has for its object the production of ornamented glass—such as tiles, panels, mosaics, and the like—for architectural purposes and other ornamental and decorative uses; and it consists in certain improvements, which will be fully disclosed in the following specification and claims.

In the accompanying drawings, which form part of this specification, Figure 1 represents a section of a tile on an enlarged or exaggerated scale; Fig. 2, a front elevation or plan view; Fig. 3, a rear elevation or plan view; Fig. 4, a section on an enlarged scale, showing a modification of the construction; Fig. 5, a front elevation or plan of the same; Fig. 6, a rear elevation or plan, and Fig. 7 a section of a modified construction.

Reference being had to the drawings and the letters thereon, A indicates a tile, panel, or mosaic which is used for the purpose of illustration, as many forms or designs may be used, and are all within the scope of my invention. The back *a* of the tile is crimped, 35 rippled, or corrugated, as shown in Figs. 1, 2, and 3, which permits the air under the tile to escape in setting it in plastic material, or roughened or stippled, as shown in Figs. 4, 5, and 6, and the front *b* is preferably smooth, 40 but may also be of the same configuration as the back, as shown in Fig. 7, or the front may have figures differing from the back.

The articles having been properly cleansed are laid upon a suitable table for the purpose 45 and heated and a solution of nitrate of silver poured on one side, preferably the back, and after having been permitted to stand a sufficient length of time to effect precipitation of the silver the remaining liquid is poured off, 50 the silvered surface thoroughly rinsed with water, and the article allowed to dry. The silver coating *c* is then covered or backed with a lead or metallic paint *d* or with asphaltum.

The tiles, panels, mosaics, or other articles are made of tinted or colored transparent or 55 translucent glass, any color, shade, or tint being used, except crystal or flint glass, and when one side is coated with the brilliant material the opposite side presents the appearance of gold, onyx, opal, mother-of-pearl 60 and other colored ornamentation upon the glass, and as light falls upon the glass the roughened surface reflects the light in a variety of angles and hues and produces a highly ornamental and pleasing effect. 65

Any of the known formulas for depositing nitrate of silver may be used.

The ornamental tiles, panels, or mosaics are designed for mural decorations, also inside and outside architectural tiles or panels 70 representing gilded iron, marble, onyx, opal, and other beautiful and precious or valuable stones, and are capable of being made in a great variety of designs by molding the molten glass into any shape desired and in a great 75 variety of colors.

Having thus fully described my invention, what I claim is—

1. A tile, panel, mosaic or other article of tinted or colored transparent material having 80 an irregular surface on one side, and one side coated with a precipitate from nitrate of silver.

2. A tile, panel, mosaic or other article of tinted or colored transparent material having an irregular surface on one side extending 85 throughout the length and width of the tile and one side covered with a brilliant material.

3. A tile, panel, mosaic or other article of tinted or colored glass having an irregular surface on both sides and one of said sides 90 coated with a brilliant material.

4. The method of ornamenting glass, which consists in tinting or coloring molten glass, forming tile, panels, mosaics or other articles by molding the article with an irregular surface and depositing silver in solution on one side of the article. 95

In testimony whereof I affix my signature in presence of two witnesses.

EDGAR J. LUTWYCHE.

Witnesses:

CHAS. H. VAN DEUSEN,  
EDWARD GEGENHEIMER.